

July 2, 1968

C. ALTMAN

3,391,373

BETA TANTALUM RESISTORS

Filed July 12, 1965

FIG. 1



FIG. 2



INVENTOR  
C. ALTMAN  
BY W. L. Williamson  
ATTORNEY

1

3,391,373

## BETA TANTALUM RESISTORS

Carl Altman, Kendall Park, N.J., assignor to Western Electric Company, Incorporated, New York, N.Y., a corporation of New York

Filed July 12, 1965, Ser. No. 470,981

6 Claims. (Cl. 338—308)

### ABSTRACT OF THE DISCLOSURE

A shaped resistive path of beta tantalum is disclosed having a greatly increased specific resistivity and a greatly improved temperature stability as compared with body-centered cubic tantalum. Beta tantalum has a specific resistivity of at least 160 micro ohms-cm. to 280 micro ohm-cm., and a temperature coefficient of resistance of from +100 p.p.m./C. ° to —100 p.p.m./C. °.

This invention relates to thin-film resistive elements and more particularly to beta tantalum thin-film resistive elements.

Reference is herewith made to the copending application, Ser. No. 448,553, of C. Altman et al. filed Apr. 5, 1965, to incorporate the application by reference thereto. This application is assigned to Western Electric Company, Inc., and to Bell Telephone Laboratories, Inc. Beta tantalum is a newly discovered material disclosed and claimed in the above-identified application which has the same gross composition as body-centered cubic tantalum (normal tantalum), but which has a different crystalline structure.

In the thin-film resistor art, resistive elements which are temperature stable and which have a high specific resistivity are highly desirable.

Temperature stability refers to the change in resistance value a resistive element experiences as a result of a change in temperature. If a resistive element has a small temperature coefficient of resistance, the resistive element does not experience a large fluctuation in resistance with changes in temperature.

The resistance value of a resistive element is determined by its physical dimensions and specific resistivity. If a resistive element has a high specific resistivity, smaller physical dimensions are required for a given resistance value. This permits a greater miniaturization of thin-film circuits.

Research resulted in the discovery that beta tantalum, although having substantially the same gross composition as normal tantalum, possesses an unexpectedly small temperature coefficient of resistance and a high specific resistivity.

It is therefore an object of this invention to provide an improved thin-film resistive element.

An additional object of this invention is to provide a temperature stable thin-film resistive element.

A further object of this invention is to provide a thin-film resistive element having a high specific resistivity.

With these and other objects in view, this invention contemplates a thin-film resistive element having a non-conductive substrate and a thin film of beta tantalum supported on the substrate, the thin film being shaped to provide a resistive path having a predetermined resistance value between its ends.

The invention may be more readily understood by reference to the description which follows when taken in conjunction with the figures in which:

FIG. 1 is a perspective view of a thin-film resistive element according to this invention; and

FIG. 2 is an enlarged sectional view shown in perspective and taken from FIG. 1 along lines 2—2.

2

Beta tantalum is most readily distinguished from normal tantalum by its crystal structure which may be observed, for example, by X-ray diffraction techniques.

An X-ray diffraction pattern for a given material is represented in conventional notation by a listing of *d*-spacings for the material in decreasing order of magnitude usually expressed in angstrom units. Each *d*-spacing of a particular material is the distance in angstrom units between individual crystal planes in a given set of parallel crystal planes.

As is well known, the term "d-spacing" derives from Bragg's law,  $\lambda=2d \sin \theta$ , where  $\lambda$  is the wavelength of the radiation reflected by parallel crystal planes,  $\theta$  is the angle of incidence (or reflection) of the radiation, and  $d$  is the distance between the parallel crystal planes.

As each crystalline material has a unique X-ray diffraction pattern, comparison of the X-ray diffraction pattern of an unknown material with the X-ray diffraction patterns for known materials, for example, as listed in published powder diffraction files, permits qualitative identification of the unknown material. Since beta tantalum possesses a unique X-ray diffraction pattern, use of this technique permits positive identification of beta tantalum. X-ray Metallography written by A. Taylor and published in 1961 by John Wiley and Sons, Inc., pp. 154—158 and 160—161, discusses X-ray diffraction patterns and their usefulness as a unique indicia for identifying materials.

Table I lists all of the *d*-spacings for beta tantalum which have been observed.

TABLE I

|    | <i>d</i> A |       |       |
|----|------------|-------|-------|
| 35 | 5.38       | 2.15  |       |
|    | 4.75       | 2.06  | 1.37  |
|    | 2.80       | 1.96  | 1.332 |
|    | 2.67       | 1.77  | 1.29  |
|    | 2.62       | 1.59  | 1.240 |
| 40 | 2.49       | 1.56  | 1.210 |
|    | 2.36       | 1.53  | 1.172 |
|    | 2.32       | 1.46  | 1.10  |
|    | 2.25       | 1.442 | 1.03  |
|    | 2.21       | 1.405 | 1.01  |

The *d*-spacings found in Table I are a compilation of *d*-spacings observed by different techniques. All of the *d*-spacings listed are observable by making direct measurements on films which have been exposed to X-rays diffracted from a sample of beta tantalum. Different techniques can be used in exposing the films from which the direct measurements are made. For example, the sample can be held stationary while the films are exposed or the sample can be oscillated. A large number of the *d*-spacings listed are obtainable by diffractometer techniques. Studies of beta tantalum by electron diffraction also confirm many of the *d*-spacings recorded in Table I.

In Table II *d*-spacings are listed which are considered to be particularly accurate. These particular *d*-spacings are confirmed by two or more different techniques.

TABLE II

|    | <i>d</i> A |       |       |
|----|------------|-------|-------|
| 60 | 5.38       | 2.32  | 1.405 |
|    | 4.75       | 2.15  | 1.332 |
|    | 2.67       | 2.06  | 1.240 |
| 65 | 2.49       | 1.77  | 1.210 |
|    | 2.36       | 1.442 | 1.172 |

The Altman et al. application mentioned above compares the composition of beta tantalum with that of normal tantalum. The results of this comparison indicate there is no gross compositional difference between beta tantalum and normal tantalum. However, research has

indicated that beta tantalum has certain very useful properties not associated with normal tantalum.

For example, the specific resistivity of beta tantalum has been discovered to be almost a magnitude greater than the specific resistivity of normal tantalum. Normal tantalum in bulk form has a specific resistivity of approximately 12 micro ohm-cm. In normal tantalum thin films, the specific resistivity is observed to be somewhat greater than that of bulk tantalum, varying between 24-50 micro ohm-cm. Beta tantalum thin films, however, have a specific resistivity of at least 160 micro ohm-cm. When the sputtering conditions set forth in the above-mentioned Altman et al. application are employed to deposit a beta tantalum film in an in-line vacuum machine of the type disclosed in the copending Charschan et al. application, Ser. No. 314,412, filed Oct. 7, 1963, new Patent No. 3,294,670, and assigned to Western Electric Company, Inc., the specific resistivity of the beta tantalum deposited lies in the range between 160 micro ohm-cm. to 280 micro ohm-cm. However, much higher values have been observed under different sputtering conditions.

In addition, beta tantalum has been discovered to have a temperature coefficient of resistance much smaller than that of normal tantalum. Normal tantalum in bulk form has a temperature coefficient of resistance of from +0.0037 to +0.0038 per centigrade degree change in temperature, or in equivalent notation, the temperature coefficient varies from +3700 to +3800 parts per million per centigrade degree (p.p.m./C.<sup>o</sup>). Using the latter notation, normal tantalum thin films have a temperature coefficient of resistance which varies from +500 to +1000 p.p.m./C.<sup>o</sup>. Beta tantalum thin films, however, are observed to have a temperature coefficient of resistance which varies from +100 p.p.m./C.<sup>o</sup> to -100 p.p.m./C.<sup>o</sup>.

A resistive element, generally indicated by the numeral 11, is illustrated in FIGS. 1 and 2. The resistive element 11 includes a nonconductive substrate 12 which supports shaped resistive paths 13-15. The nonconductive substrate 12 may be of glass, ceramic, or any other suitable material. The resistive paths 13-15 may have any suitable configuration. For example, resistive path 13 illustrates a straight line configuration whereas resistive paths 14 and 15 illustrate tortuous configurations.

As is well known, the resistance value of a given resistive element is a function of the physical dimensions and specific resistivity of its resistive path. This relationship may be expressed by the formula  $R = \rho l / wt$ , where  $R$  is the resistance value,  $\rho$  is the specific resistivity,  $l$  is the length,  $t$  is the thickness and  $w$  is the width of the resistive path.

For example, the resistance value  $R$  of a resistive element of normal tantalum having a specific resistivity  $\rho$  of 50 micro ohm-cm., a length  $l$  of 9 cm., a thickness  $t$  of 2,000 angstroms ( $2.0 \times 10^{-5}$  cm.) and a width  $w$  of 0.015 cm. is 1500 ohms. In contrast, resistance value  $R$  of a resistive element of beta tantalum having the same dimensions is 6,000 ohms where the specific resistivity  $\rho$  is 200 micro ohm-cm. For example, a 1500 ohm beta tantalum resistive element having a specific resistivity of 200 micro ohm-cm. and the same width and thickness as the normal tantalum resistive element would have a length of only 2.25 cm. as contrasted with the length of 9 cm. for the normal tantalum resistive element. Accordingly, a beta tantalum thin-film resistive element having the same resistance value as a normal tantalum thin-film resistive element is much smaller in physical size.

In addition, beta tantalum resistive elements experience a much smaller change in resistance value with fluctuations in temperature. The change in resistance value  $\Delta R$  is expressed by the formula  $\Delta R = \alpha R \Delta T$  where  $\alpha$  is the temperature coefficient of resistance,  $R$  is the resistance value at some arbitrary base temperature, and  $\Delta T$  is the change in temperature from the base tempera-

ture. Where the base temperature is taken at 0° C.,  $\Delta T$  is simply the temperature of the resistive element.

For example, the change in resistance value  $\Delta R$  of a 5,000-ohm resistive element of normal tantalum having a temperature coefficient of resistance  $\alpha$  of +500 p.p.m./C.<sup>o</sup> is 250 ohms for a change in temperature  $\Delta T$  of 100° C. In contrast, the change in resistance value  $\Delta R$  of a 5,000-ohm resistive element of beta tantalum having a temperature coefficient of resistance  $\alpha$  of +100 p.p.m./C.<sup>o</sup> is 50 ohms for a change in temperature  $\Delta T$  of 100° C. Accordingly, beta tantalum thin-film resistive elements are much more temperature stable than those of normal tantalum.

As the resistive value of resistive elements is a function of their physical dimensions, it is necessary to properly shape a resistive path to obtain a desired resistance value. A highly suitable technique for shaping a beta tantalum resistive path includes depositing a continuous film of beta tantalum on a nonconductive substrate. The sputtering conditions are set forth in the above-mentioned Altman et al. application for depositing such a continuous film of beta tantalum on a substrate in an in-line vacuum machine of the type disclosed in the above-mentioned Charschan et al. application. The beta tantalum films deposited are adherent uniform films which are suitable for the manufacture of resistive elements.

The thickness of the continuous film may be controlled by the length of time a substrate is exposed to a sputtering source. To form a resistive path from a continuous film having the desired thickness, it is only necessary to shape the resistive path to the desired length and width from the continuous film. This may be readily accomplished with conventional photoetching techniques.

In generating circuit patterns, or in this context shaping resistive paths, by photoetching, a light-sensitive emulsion or resist is applied to the continuous film. The resist is then over-baked to set the resist properly. The resist is subsequently exposed to an ultraviolet light source through a mask which is a negative of the desired circuit pattern. The exposed areas of the resist are polymerized by the ultraviolet light to make them resistant to attack by solvents and acids. The resist is then soaked in a solvent which removes the unexposed resist. The resist is again oven-baked to remove any solvent and to harden the resist.

By applying a suitable acid to the continuous film, those areas of the film which are protected by the polymerized resist are left on the substrate while the unprotected areas are removed by the acid. In this manner, circuit patterns or as in this case shaped resistive paths, may be formed from a continuous film.

Any suitable resist may be used such as KMER (Kodak Metal Etch Resist) and KPR (Kodak Photo Resist). A mixture of silane and toluene is a suitable solvent for use with KMER and KPR. Beta tantalum is readily etched by a mixture of nitric and hydrofluoric acids in the same manner in which normal tantalum is etched.

The effective dimensions of a resistive element may also be reduced subsequent to shaping a desired resistive path by converting a portion of the resistive path to an oxide. A suitable anodization process for accomplishing this is disclosed in U.S. Patent 3,148,129 assigned to Bell Telephone Laboratories, Inc. This process is suitable for anodizing beta tantalum resistive elements and permits the fabrication of high precision resistive elements.

Subsequent to shaping the desired resistive paths from the continuous film, metals are deposited on the substrate to complete circuit wiring and to provide contact areas for lead attachment. The metals used should exhibit a combination of good adherence, high conductivity and resistance against atmospheric oxidation. Typically, a nickel-chromium alloy is deposited directly on the substrate for good adherence, followed by a film of copper for high conductivity and solderability. Finally, a film of gold is added to provide resistance to oxidation. These

metals may be successively deposited by evaporation through a suitably prepared mechanical mask.

Contact pads 17-19 illustrate how these metal areas may be used. The contact pad 17, for example, terminates resistive path 13 and provides an area to which a lead 21 is soldered. The contact pads 18 and 19 terminate the resistive paths, to provide areas suitable for the attachment of leads 21, and to interconnect the resistive paths. As will be obvious to one skilled in the art, any desired grouping of resistive paths may be provided.

Any technique suitable for generating shaped resistive paths from normal tantalum may also be employed in shaping beta tantalum resistive paths. For example, beta tantalum may be deposited onto a substrate through a mask which defines the desired pattern. This eliminates the necessity of removing undesired portions of a continuous film by photoetching techniques. In addition, contact pads and internal circuit interconnection may be deposited in a continuous film followed by the removal of undesired portions by photoetching techniques.

What is claimed is:

1. A thin-film resistive element comprising:  
a nonconductive substrate; and  
a thin-film resistive material supported on the substrate  
and shaped to provide a resistance path of predetermined resistance value between its ends, said resistive material further comprising beta tantalum.
2. A thin-film resistive element comprising:  
a nonconductive substrate;  
two spaced contact pads supported on the substrate; and  
a thin-film resistive material supported on the substrate  
to interconnect the contact pads and shaped to provide a resistance path of predetermined resistance value between the pads, said resistive material further comprising beta tantalum.
3. A thin-film resistive element comprising:  
a nonconductive substrate;  
two spaced contact pads supported on the substrate; and  
a thin-film resistive material supported on the substrate  
to interconnect the contact pads and forming a tortuous resistive path between the contact pads having a predetermined resistance value, said resistive material further comprising beta tantalum.

5

10

15

20

25

30

35

40

4. A thin-film resistive element comprising:  
a nonconductive substrate; and  
a thin-film resistive material supported on the substrate  
and shaped to provide a resistance path of predetermined resistance value between its ends, said resistive material being identifiable by the following *d*-spacings in angstrom units: 5.38, 4.75, 2.67, 2.49, 2.36, 2.32, 2.15, 2.06, 1.77, 1.442, 1.405, 1.332, 1.240, 1.210, and 1.172.
5. A thin-film resistive element comprising:  
a nonconductive substrate;  
two spaced contact pads supported on the substrate; and  
a thin-film resistive material supported on the substrate  
to interconnect the contact pads and shaped to provide a resistance path of predetermined resistance value between the pads, said resistive material being defined by the following *d*-spacings in angstrom units: 5.38, 4.75, 2.67, 2.49, 2.36, 2.32, 2.15, 2.06, 1.77, 1.442, 1.405, 1.332, 1.240, 1.210, and 1.172.
6. A thin-film resistive element comprising:  
a nonconductive substrate;  
two spaced contact pads supported on the substrate; and  
a thin-film resistive material supported on the substrate  
to interconnect the contact pads and forming a tortuous resistive path between the contact pads having a predetermined resistance value, said resistive material being defined by the following *d*-spacings in angstrom units: 5.38, 4.75, 2.80, 2.67, 2.62, 2.49, 2.36, 2.32, 2.25, 2.21, 2.15, 2.06, 1.96, 1.77, 1.59, 1.56, 1.53, 1.46, 1.442, 1.405, 1.37, 1.332, 1.29, 1.240, 1.210, 1.172, 1.10, 1.03, and 1.01.

#### References Cited

##### UNITED STATES PATENTS

3,275,915 9/1966 Harendza-Harinxma ... 317—258

##### FOREIGN PATENTS

991,649 5/1965 Great Britain.

RICHARD M. WOOD, *Primary Examiner.*

J. G. SMITH, *Assistant Examiner.*